

G. ISSLER.  
METHOD OF DENSIFYING FUSIBLE EXPLOSIVE NITRO BODIES.  
APPLICATION FILED JAN. 13, 1912.

1,074,263.

Patented Sept. 30, 1913.

FIG. 1.



FIG. 2.

WITNESSES:

M. M. Hamilton  
E. E. Mall

INVENTOR

Gottbold Issler  
BY Frank S. Buser  
ATTORNEY.

# UNITED STATES PATENT OFFICE.

GOTTHOLD ISSLER, OF WAHN, GERMANY, ASSIGNOR TO E. I. DU PONT DE NEMOURS POWDER COMPANY, OF WILMINGTON, DELAWARE, A CORPORATION OF NEW JERSEY.

## METHOD OF DENSIFYING FUSIBLE EXPLOSIVE NITRO-BODIES.

1,074,263.

Specification of Letters Patent. Patented Sept. 30, 1913.

Application filed January 13, 1912. Serial No. 671,096.

To all whom it may concern:

Be it known that I, GOTTHOLD ISSLER, a subject of the Emperor of Germany, residing at Wahn, in the German Empire, have 5 invented a new and useful Improvement in Methods for Densifying Fusible Explosive Nitro-Bodies, of which the following is a full, clear, and exact description, reference being had to the accompanying drawings, 10 which form a part of this specification.

The general method used for densifying explosive nitro bodies which consists in pressing by mechanical means the powdered material in special presses is very inconvenient and expensive. For this reason a 15 large number of other methods have been proposed, all of which aim at rendering the densifying of nitro bodies less expensive and at simplifying same. It is especially important to densify nitro bodies which are to be 20 used for charges of projectiles, mines and torpedoes, because, with a higher density, the efficiency is greater and a denser nitro body is less sensitive against outside influences and influences during the shot.

Most of the charges for projectiles are cast in paste-board shells or paste board boxes which are sealed water-tight, and the paste-board boxes must be entirely filled by 30 the nitro body so as to prevent the formation of dust or allowing the charge to move in the box during the shot. Some organic nitro bodies possess the property of contracting during the chilling, thus producing 35 an interstice between the charge and the paste-board box, which for reasons of safety must be eliminated.

I have discovered a method which produces, in a most simple manner, as high a 40 density as possible of organic nitro-bodies used for charges of projectiles, etc., and which effects a tight bearing of these charges against the walls of the paste-board box.

I have discovered that if the upper part 45 of the "lost head" (i. e. that part of the nitro body above the box when the process is finished and which is removed) be maintained liquid, while by means of a piston or other compressive force, pressure is transmitted through the liquid layer to the charge, the highest density of the nitro body will be produced, the same will entirely fill the box and empty spaces in the cast will be avoided.

I will now describe an apparatus for carrying out my method, which apparatus is shown in the accompanying drawing, which shows a front elevation, partially in section, of such apparatus.

A paste-board box *a* is located in a mold *b*, the latter being somewhat higher than the paste-board box.

*c* is an iron pipe which rests on the top of the box *a* and is closely surrounded at this lower portion by the mold *b*. On the upper border of the pipe *c* rests a circular metal plate *e* upon which a top piece *d* is welded. An annular washer *h* for the purpose of rendering the joint tight is inserted between the top of the pipe *c* and the metal circular plate *e*. This top piece *d* forms a jacketed hollow cylinder which can be heated by means of steam or by means of another heat generator, and the cylinder is for this purpose, provided with a steam inlet *i* and a steam outlet *h*. The mold *b* and the intermediate piece *c* are by means of the bolts *f* fastened between the bottom plate *m* and the metal circular plate *e* in such manner that the whole apparatus can be rendered tight. On the plate *e*, on opposite sides of the top piece *d*, are posts *n*, connected, above the top-piece, by the cross-plate *n'*. In the top piece *d* is a piston *g*. The piston rod *g'* extends up through the cross-plate *n'*, its threaded upper end carrying a hand-wheel *r*. A valved pipe *o* extends into the lower part of the top piece. The apparatus rests on the bottom of a vessel *p* adapted to contain a cooling liquid. By means of the hand-wheel *r*, the piston *g* can be moved down and thus a pressure can be brought to bear upon the upper part of the nitro body which is maintained liquid.

The operation of the apparatus is very simple. The paste-board box *a* is placed in the mold *b*, the pipe *c*, plate *e* and top piece *d* are placed in position and rendered tight and then the liquid nitro body is introduced. Connection is then made with the steam line, the heat is turned on, and the piston *g* is screwed down, in which operation the nitro body itself serves as lubricant. The introduction of the liquid is effected by removing the cover *d'* of the top piece *d* and, by means of the hand wheel *r*, raising the piston *g* until it is withdrawn from the interior of the top piece. The pressure, of course, can

be brought about in any other desired manner, for instance, by means of a weight or by compressed air. It has been found to be of advantage to cool the mold about to the upper border of the paste-board box. After the operation the upper part of the lost head that has been maintained liquid is withdrawn through the pipe *o*.

This method actually effects the high density (1.60 to 1.62) and an entire filling of the paste-board box with the nitro body. Empty spaces in the cast are impossible since the liquid nitro body under pressure fills any such spaces.

15 I do not claim herein the apparatus herein described, as the same forms the subject-matter of a separate application filed by me of even date herewith, Serial No. 671,097.

Having now fully described my invention, 20 what I claim and desire to protect by Letters Patent is:

1. The method for densifying fusible explosive nitro bodies, which consists in casting the main body with an integral part 25 projecting beyond the same to form the lost head and maintaining in a liquid state the part of the lost head more remote from the

main body while applying pressure through the liquid layer to the charge.

2. The method for densifying fusible explosive nitro bodies cast in containers which consists in charging the container and allowing an integral part of the nitro body to project above the container to form the lost head and maintaining the upper part of the lost head liquid while applying pressure through the liquid layer to the charge.

3. The method for densifying fusible explosive nitro bodies which consists in applying heat to and thereby maintaining fused or liquid one end of the charge, and applying pressure to the charge through the medium of the part maintained liquid while gradually chilling the part of the charge more remote from the part maintained liquid.

In testimony of which invention, I have hereunto set my hand, at Cologne, Germany, on this 15th day of December, 1911.

GOTTHOLD ISSLER.

Witnesses:

ANIS VANDORY,  
BESSIE F. DUNLAP.